

Sept. 23, 1941.

G. S. LEWIS

2,256,947

WHEEL RIM AND METAL TREATING METHOD

Filed Jan. 2, 1940



Inventor:  
George S. Lewis,  
By Chittom, Miles, Davies, Kirch & Dawson,  
Attorneys

## UNITED STATES PATENT OFFICE

2,256,947

WHEEL RIM AND METAL TREATING  
METHOD

George S. Lewis, Evanston, Ill.

Application January 2, 1940, Serial No. 312,129

2 Claims. (Cl. 148—10)

This invention relates to a wheel rim and to a metal treating method. The method may be used not only in forming the wheel rim but also in forming treated materials used in the manufacture of other products.

In the manufacture of wheel rims, it has been necessary to employ metal strips of relatively soft or low temper in order to enable the edge portions to be rolled to form beads. Should a metal strip of relatively high temper be used, the edge portions when rolled to form the beads split and break. It is desirable, however, to have the rim formed, in so far as is possible, of metal of relatively high temper in order to reduce the amount of metal used and in order to provide the rigidity desired for the rim.

An object of the present invention is to provide a method by which a rim formed of relatively high temper metal may be produced while at the same time forming beads thereon without difficulty. A further object is to provide a rim having beads at the edges thereof formed of annealed metal, the remaining portion of the rim being of relatively high temper metal. A further object is to provide a method of treating metal strips of relatively high temper so that edge portions or other areas thereof are annealed or otherwise treated so as to permit rolling or other manipulation thereof. Other specific objects and advantages will appear as the specification proceeds.

The invention is illustrated, in a preferred embodiment, by the accompanying drawing, in which—

Figure 1 is a side view in elevation of apparatus suitable for the practice of my invention; Fig. 2, a top plan view of the same; Fig. 3, a broken perspective view of a strip of metal treated in accordance with my invention; and Fig. 4, a transverse sectional view of the rim formed in accordance with my invention.

In the illustration given, 10 designates a standard supporting a trunnion-equipped reel 11 upon which is wound a long strip of metal 12. The reel 11 is shown equipped with handles 13 which may be employed in the winding of the metal thereon or the dispensing of the same from the spool or reel.

Just ahead of the standard 10 is a frame 14 consisting of three standards, each supporting a platform 15. Mounted on each of the platforms 15 are a pair of feed rollers 16 spaced apart to receive the strip metal 12. The feed or drive rollers 16 are each mounted upon a shaft 17 journaled within a bearing 18 secured to the frame 55

14. The shaft 17 is driven by any suitable means (not shown).

Spaced between the standards 14 are transformers 19 and 20 which are of well-known construction and need not be described in detail.

5 Transformer 19 is provided with a pair of spaced roller electrodes 21 adapted to receive between them the metal strip 12. The roller electrodes 21 are of the type usually employed for seam welding and need not be described in detail. Each roller is equipped with an edge portion which directly engages the edge portions of the metal strip 12.

10 The transformer 20 is likewise equipped with roller electrodes 22 which are spaced apart to receive the metal strip 12.

15 The metal strip 12 is, after the treating operation, wound upon a second spool or reel 23 equipped with handles 24 and the journal 25, the journal 25 being supported upon a bearing 26 provided by the standard 21.

20 In the operation of the apparatus, a strip of metal 12 is fed from the spool 11 between the feed rollers 16 carried by the three platforms 15, the electrodes 21 and 22 being spaced at such distance from each other as to engage opposite edge portions of the strip 12. It will be understood that the electrodes are adjustable laterally so as to enable them to engage strips of metal of varying widths. The strip of metal, after being fed 25 between the electrodes, is wound upon the reel 23.

25 In order to anneal the edge portions of the strip without substantially affecting the temper of the remaining portion of the strip, it is important that the strip 12 be advanced at such a speed as to maintain the temperature of the edge portions of the strip at an annealing temperature and without allowing the temperature of the edge portions of the strip to exceed these temperatures. In other words, if the metal were allowed 30 to remain between the electrodes for the usual length of time, a welding temperature would be reached, but where the strip is moved forward at a predetermined speed, the temperature created in the metal does not exceed a cherry red 35 temperature. It is found that, where the speed of movement of the metal is thus coordinated with the usual roller electrodes employed for making seam welds, that a quick heating of the areas along the edges of the metal to an annealing 40 temperature is effected without causing this temperature to extend to the remaining portions of the metal. As a result, the major portion of the strip retains its initial temper, while the edge portions have their temper considerably reduced.

45

By way of example, it is found that where a half hard cold rolled sheet steel .050 thick is treated in the manner described, the temper midway between the edges on some samples was approximately 75B Rockwell while the temper closely adjacent the edge was 36B Rockwell. Similarly, when strips of full hard cold rolled sheet steel .050 thick were treated as above described, the temper midway between the edges was approximately 94B Rockwell, and the temper closely adjacent the edge 57B Rockwell. In another case, the temper midway between the edges was 96B Rockwell while the temper adjacent the edge was 61B Rockwell. In still another case, the temper midway between the edges was 96B Rockwell, while the temper adjacent the edge was 60B Rockwell.

In Figure 3 is shown a strip of metal 28 having all edge portions 29 thereof annealed in accordance with the method described. The soft edge portions 29 are readily rolled to form the beads 30 of the tire rim 31, shown in Fig. 4.

By following the method described, it is possible to form rims of relatively thin metal of high temper, while at the same time the beads 30 may be readily produced without danger of splitting.

It will be understood that the method is not limited to the treatment of edge portions only. If it is desired to bend other portions of the metal, such as, by creasing the same, and where an annealed area is required, the annealed area may be produced at any point desired upon the metal strip 12 by adjusting the position of the metal or electrodes. I have found it particularly useful, however, in the formation of rims because of the ease with which the edge portions may be

treated without affecting in any substantial degree the temper of the remaining portion of the metal. It will be noted that the edge portions 29 are separated by the main width of the metal.

5 While in the foregoing specification, I have set forth certain details of apparatus and certain steps in the method, it will be understood that these are for the purpose of illustration only and that such details and step-sequences may be varied widely by those skilled in the art without departing from the spirit of my invention.

I claim:

1. The method of annealing areas of a relatively high temper metal strip comprising subjecting said areas to contact with the electrodes of an electric welding device long enough to raise said areas to an annealing temperature, causing said areas to pass beyond the heating zone after having reached the proper temperature for annealing, thereby preventing the remaining areas from becoming annealed, and slowly cooling said areas.

15 2. The method of annealing the opposite edge portions of a high temper metal strip comprising subjecting each of said edge portions to contact with a pair of spaced electrodes of an electric welding device long enough to raise each edge portion to an annealing temperature, the heating of said edge portions being carried on simultaneously, causing said edge portion to pass beyond the said device after having reached the proper temperature for annealing, thereby preventing the remaining portions from becoming annealed, and slowly cooling said edge portions.

35

GEORGE S. LEWIS.